

A. P. CRAFT.  
PROCESS OF TREATING ZINC ORES.  
APPLICATION FILED JUNE 23, 1917.

1,295,857.

Patented Mar. 4, 1919



WITNESS.

Walter H. Troost

INVENTOR

INVENTOR  
Augustus P. Craft  
BY  
Broderick & Deshields  
ATTORNEYS

# UNITED STATES PATENT OFFICE.

AUGUSTUS P. CRAFT, OF GALENA, ILLINOIS.

## PROCESS OF TREATING ZINC ORES.

1,295,857.

Specification of Letters Patent. Patented Mar. 4, 1919.

Application filed June 23, 1917. Serial No. 176,483.

To all whom it may concern:

Be it known that I, AUGUSTUS P. CRAFT, a citizen of the United States, residing at Galena, Jo Daviess county, and State of 5 Illinois, have invented and discovered certain new and useful Improvements in Processes of Treating Zinc Ores, of which the following is a specification.

My invention relates to processes of treating 10 zinc ores and its object is to obtain a yield of higher quality and in which particularly the impurities which are in such fine, pulverulent condition that they can not be effectively and economically separated from the ore according to present 15 processes, may be eliminated.

With this object in view my process is embodied in the steps hereinafter described, and an apparatus for carrying out such 20 process is illustrated in the accompanying drawings.

In these drawings, Figure 1 is a longitudinal sectional elevation of a zinc ore magnetic separating mechanism, Fig. 2 a plan view thereof partly in section, Fig. 3, a section on line 3—3 of Fig. 1, and Fig. 4, a detail perspective of the fine mesh screen.

The quality of zinc ore is determined mainly by the percentage of metallic zinc 30 contained therein and the prices per ton of the zinc are measured by these percentages. In zinc sulfid ores, such as are found in the Wisconsin, Galena and Joplin districts, the principal impurities retained in the ore, 35 after roasting and magnetic separation, are lime and iron pyrites. These impurities exist mainly in a fine condition in the ore and are carried by and form part of the fine body of dust or powder to which part of the 40 ore is reduced in its various treatments of crushing, concentrating, drying, roasting, shaking and separating. My invention consists in separating this finer body of ore from the mass after the steps of roasting, 45 and separation of the larger particles of iron therefrom, for the purpose of carrying with it the lime, fine iron pyrites or flour iron and other fine impurities, and then subsequently and separately treating this 50 body according to well known methods to separate the impurities therefrom.

The drawings show an apparatus designed to carry out these processes. In these drawings 1, indicates a magnetic separator 55 to which the ore is conducted after it has been concentrated and dried and roasted or

oxidized, and 2, indicates an agitating, gravity-feed, inclined table to which the ore is fed. Above this table depend magnets 3, which serve to attract and thus separate 60 the larger particles of iron from the ore, such particles being attracted to and conveyed away by means of conveying belts 4, around the magnets. A magnetic separator of this kind is well known. This magnetic 65 separator is capable of extracting only the larger particles of iron and of course is ineffective to separate the lime from this ore.

In ore separating mills a plurality of such 70 separators with their tables are employed.

In carrying out my invention, at the lower discharge end of the table 2, I provide screen 5, which is preferably of about 50 mesh and of such fine degree of mesh as to permit only the small, substantially pulverulent particles of the ore, such as are capable of separation from the impurities by means of the oil flotation process or the slime table process, and incapable of separation by the dry process, to pass through 80 the same. This screen is agitated, to aid in the sifting of the ore and to this end the screen may be made part of or attached to the shaking table 2, as shown. The fine body of ore that passes through this fine mesh screen 85 will carry with it the lime, iron pyrites and similar fine impurities that are mixed with and carried along by the dust or pulverized body of the mass of ore. The mass of small particles thus collected is then capable of 90 ready treatment by a wet process, such as the slime table method which is well known and which may be successfully used to extract the lime and pyrites and other impurities therefrom, and which process can 95 not be successfully used with the ore in the form of the larger particles.

In the ordinary zinc dressing operation, this fine body of ore is carried along with the coarse particles and the fine impurities 100 will be retained, owing to the fact that they can not be separated by the dry process, and they tend to greatly depreciate the quality of the ore, and to lower its percentage of metallic zinc, and therefore greatly decrease 105 the price per ton that is paid therefor as compared with ores which are free from such impurities. The process therefore not only eliminates the mass of fine ore from the coarser particles and raises the percentage 110 of the latter mass, but also enables the body of fine material to be effectively dressed so

as to recover quite a large percentage of zinc therefrom.

Having thus described my invention, what I claim is:—

5 The process of dressing roasted zinc ores which consists in separating the larger particles of iron therefrom by magnetic separation, then immediately subjecting the ore as it passes from said treatment to an agitating and screening action on a screen of not less than fifty mesh to the inch to separate and collect the fine ores therefrom and then sub-

jecting such collected body of particles of ore to a wet separation process to remove the lime, iron pyrites and other impurities. 15

In witness whereof, I have hereunto set my hand and seal at Indianapolis this 19th day of June, A. D. nineteen hundred and seventeen.

AUGUSTUS P. CRAFT. [L. S.]

Witnesses:

H. P. DOOLITTLE,  
M. L. WHEELER.